

Sept. 23, 1924.

1,509,617

K. A. SODERSTROM

METHOD OF CUTTING BARS FROM CENTRIFUGAL CASTINGS

Filed April 17, 1923

2 Sheets-Sheet 1



FIG. 1.



FIG. 2.

WITNESS:

Bob Kitchel.

INVENTOR

Karl A. Soderstrom

BY

Frank S. Buser  
ATTORNEY

Sept. 23, 1924.

1,509,617

K. A. SODERSTROM

METHOD OF CUTTING BARS FROM CENTRIFUGAL CASTINGS

Filed April 17, 1923

2 Sheets-Sheet 2



FIG. 3.



FIG. 4.



FIG. 5.



FIG. 6.

WITNESS:

Bob R. Kitchel

INVENTOR

Karl A. Soderstrom

BY

Frank J. Bussar

ATTORNEY.

Patented Sept. 23, 1924.

1,509,617

# UNITED STATES PATENT OFFICE.

KARL A. SODERSTROM, OF PHILADELPHIA, PENNSYLVANIA.

## METHOD OF CUTTING BARS FROM CENTRIFUGAL CASTINGS.

Application filed April 17, 1923. Serial No. 632,716.

To all whom it may concern:

Be it known that I, KARL A. SODERSTROM, a citizen of the United States, residing at Philadelphia, county of Philadelphia, and 5 State of Pennsylvania, have invented a new and useful Improvement in Methods of Cutting Bars from Centrifugal Castings, of which the following is a full, clear, and exact description, reference being had to the 10 accompanying drawings, which form a part of this specification.

My invention relates to a novel method of cutting bars from centrifugally cast shells or ingots.

15 In the manufacture of various products of steel, it is found desirable to have the carbon content vary throughout the product. For example, in a steel rail, it is desirable that the head of the rail be relatively high in carbon, while the foot may be relatively low in carbon. In the manufacture of plow shares, it is desirable to leave one face of the share high in carbon and the other face relatively low in carbon, 20 which is at present effected by forming the share of two plates, one of relatively high carbon and the other of relatively low carbon, secured together.

Further, in the manufacture of springs, 30 it is found desirable that one portion of the spring be higher in carbon than another.

Now it is the object of my invention to provide a method whereby bars or billets may be produced which will enable the 35 production of articles having varying carbon content. More particularly, it is the object of my invention to provide a method of producing bars, wherein the carbon content varies, from centrifugally cast shells or 40 ingots.

Having now indicated in a general way the nature, purpose and advantages of my invention, I will now proceed to a detailed description thereof with reference to the 45 accompanying drawings, in which:

Fig. 1 is a diagrammatic view of a centrifugal casting apparatus with a casting therein.

Fig. 2 is a diagrammatic view of a cutter 50 and supporting roll in operative relation to a centrifugally cast shell.

Fig. 3 is a diagrammatic view of apparatus for spirally cutting a shell and straightening a spiral.

55 Fig. 4 is a cross-sectional view of a bar for forming a rail.

Fig. 5 is a cross-sectional view of a bar for forming a spring leaf.

Fig. 6 is a cross-sectional view of a plate for forming a plow share.

*a* represents a centrifugal mold provided with top and bottom covers *b*, *b'* formed so as to produce a shell or casting *c* having formed at its ends an abruptly stopped spiral, as indicated at *d*. The mold is adapted to be supported for rotation by means of a fly wheel *e* in engagement with a friction ring *f* on the mold.

The shell or casting *c* is formed in the mold under the influence of centrifugal force, and its composition, so far as carbon content is concerned, varies from a relatively high carbon content adjacent the inner face of the wall of the shell to a relatively low carbon content adjacent the outer face of the wall, the intermediate portion varying in carbon content from the maximum to the minimum. In Fig. 1 I have indicated the zone of relatively high carbon by the letter *g*, the zone of relatively low carbon by the letter *h*, and the intermediate zone by the letter *i*.

In accordance with my method, the shell or casting *c*, after having been cast, is removed from the mold *a* and one of its ends supported upon a supporting roll *j* mounted upon a shaft *k* and provided with an end flange *l* adapted to engage the end of the shell. Cooperating with the supporting roll is a cutter *m*, mounted upon a shaft *n*, and adapted to engage the abruptly stopped spiral formed on the end of the shell and cut the shell spirally from end to end. The shaft *k* of the supporting roll may be driven through suitable gears from a shaft *o*, which in turn is driven through a ring gear *p*.

The shaft *n* is supported at one end by a bracket *q* pivoted on shaft *r* and at the other end by strap *s* pivotally secured to a bearing *t*. The shaft *n* is driven by means of a ring gear *p'* and as will be observed may be swung on the shaft *r* to enable adjustment of the cutter.

The spiral *u* cut from the shell is received between guide *v* and guided between a pair of rolls *w*, which act to straighten and shape the spiral to produce a bar *x* for the fabrication of a rail or a bar *y* for the fabrication of spring leaves, or a bar *z* for the fabrication of, for example, a plow share.

It will now be observed that by virtue of cutting the shell *e* spirally and straighten-

ing the spiral, a bar is produced having differential carbon content and from which may be produced rails having a high carbon head and a relatively low carbon foot. It 5 will be obvious that such a bar will lend itself to the fabrication of a plow share having one face of high carbon and the other face of low carbon, thus avoiding the necessity of the use of two plates.

10 It will be obvious that my invention is not limited to any particular use of the bar produced, as many uses therefor will commend themselves.

Having now fully described my invention, 15 what I claim and desire to protect by Letters Patent is:

1. The method of producing bars consisting in spirally cutting a centrifugally cast hollow ingot.

20 2. The method of producing bars consisting in spirally cutting a centrifugally cast hollow ingot and straightening the spiral, all while the metal is in a heated condition.

25 3. The method of producing steel bars having a relatively high carbon content adjacent one surface and a relatively low carbon content adjacent the opposite surface consisting in forming a cylindrical shell the carbon content of the walls of 30 which vary in the direction of the radii of the shell and spirally cutting the shell.

4. The method of producing steel bars having a relatively high carbon content adjacent one surface and a relatively low carbon content adjacent the opposite surface 35 consisting in spirally cutting a shell formed by centrifugally casting carbon steel.

5. The method of producing steel bars having a relatively high carbon content adjacent one surface and a relatively low carbon content adjacent the opposite surface consisting in centrifugally casting a shell of carbon steel, removing the shell from the mold, and spirally cutting the shell. 40 45

6. The method of producing steel bars having a relatively high carbon content adjacent one surface and a relatively low carbon content adjacent the opposite surface consisting in forming a cylindrical shell 50 having an abruptly stopped spiral at one end, spirally cutting the shell, and straightening the spiral.

7. The method of producing articles having a differential carbon content consisting 55 in centrifugally casting a shell, spirally cutting the shell, straightening the spiral to form a bar, and working the bar to produce the article.

In testimony of which invention I have 60 hereunto set my hand, at Pittsburgh, on this twelfth day of April, 1923.

KARL A. SODERSTROM.